



US007767373B2

(12) **United States Patent**  
**Goodman et al.**

(10) **Patent No.:** **US 7,767,373 B2**  
(45) **Date of Patent:** **Aug. 3, 2010**

(54) **IMAGING MEMBER HAVING HIGH MOLECULAR WEIGHT BINDER**

(75) Inventors: **Donald J. Goodman**, Pittsford, NY (US); **Satish Parikh**, Rochester, NY (US); **Edward F. Grabowski**, Webster, NY (US); **Kathleen M. Carmichael**, Williamson, NY (US); **David M. Skinner**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 953 days.

(21) Appl. No.: **11/508,484**

(22) Filed: **Aug. 23, 2006**

(65) **Prior Publication Data**

US 2008/0050665 A1 Feb. 28, 2008

(51) **Int. Cl.**

**G03G 5/10** (2006.01)

(52) **U.S. Cl.** ..... **430/59.6**; 430/69; 399/159

(58) **Field of Classification Search** ..... 430/59.6, 430/69; 399/159

See application file for complete search history.

(56) **References Cited**

U.S. PATENT DOCUMENTS

|             |        |                  |
|-------------|--------|------------------|
| 3,121,006 A | 2/1964 | Middleton et al. |
| 3,820,989 A | 6/1974 | Rule et al.      |
| 3,837,851 A | 9/1974 | Shattuck et al.  |
| 3,895,944 A | 7/1975 | Wiedemann et al. |
| 4,150,987 A | 4/1979 | Anderson et al.  |
| 4,245,021 A | 1/1981 | Kazami et al.    |
| 4,256,821 A | 3/1981 | Enomoto et al.   |

|                  |         |                             |
|------------------|---------|-----------------------------|
| 4,265,990 A      | 5/1981  | Stolka et al.               |
| 4,278,746 A      | 7/1981  | Goto et al.                 |
| 4,286,033 A      | 8/1981  | Neyhart et al.              |
| 4,291,110 A      | 9/1981  | Lee                         |
| 4,297,426 A      | 10/1981 | Sakai et al.                |
| 4,315,982 A      | 2/1982  | Ishikawa et al.             |
| 4,338,387 A      | 7/1982  | Hewitt                      |
| 4,338,388 A      | 7/1982  | Sakai et al.                |
| 4,385,106 A      | 5/1983  | Sakai                       |
| 4,387,147 A      | 6/1983  | Sakai                       |
| 4,399,207 A      | 8/1983  | Sakai et al.                |
| 4,399,208 A      | 8/1983  | Takasu et al.               |
| 4,587,189 A      | 5/1986  | Hor et al.                  |
| 4,654,284 A      | 3/1987  | Yu et al.                   |
| 4,664,995 A      | 5/1987  | Horgan et al.               |
| 4,988,597 A      | 1/1991  | Spiewak et al.              |
| 5,244,762 A      | 9/1993  | Spiewak et al.              |
| 5,756,245 A      | 5/1998  | Esteghamatian et al.        |
| 6,124,514 A      | 9/2000  | Emmrich et al.              |
| 2004/0018440 A1  | 1/2004  | Lin et al.                  |
| 2004/0115545 A1  | 6/2004  | Horgan et al.               |
| 2004/0126684 A1* | 7/2004  | Horgan et al. .... 430/58.3 |
| 2005/0053845 A1* | 3/2005  | Becker et al. .... 430/5    |
| 2005/0053854 A1* | 3/2005  | Pai et al. .... 430/58.65   |
| 2005/0233229 A1* | 10/2005 | Yu et al. .... 430/56       |

\* cited by examiner

*Primary Examiner*—John L Goodrow

(74) *Attorney, Agent, or Firm*—Pillsbury Winthrop Sha Pittman LLP

(57) **ABSTRACT**

Imaging members useful in electrostatographic apparatuses, including printers, copiers, other reproductive devices, and digital apparatuses. More particularly, imaging members having a binder of high molecular weight that is included in one or more layers of an imaging member to impart coating consistency and to provide for increased mechanical strength and improved wear.

**18 Claims, 1 Drawing Sheet**



FIG. 1



FIG. 2

## IMAGING MEMBER HAVING HIGH MOLECULAR WEIGHT BINDER

## BACKGROUND

Herein disclosed are imaging members useful in electrostaticographic apparatuses, including printers, copiers, other reproductive devices, and digital apparatuses. Some specific embodiments are directed to imaging members that have a polycarbonate binder with a specific configuration dispersed or contained in one or more layers of the imaging member. The polycarbonate used as the binder has a relatively high molecular weight and possesses solubility in specific solvents to impart uniform coatings and mechanical robustness. In addition, the polycarbonate may provide an imaging member with longer life and reduced marring, scratching, abrasion and wearing of the surface. Thus, incorporation of the polycarbonate binder into one or more layers of the imaging member provides for increased mechanical strength and improved wear to the imaging member.

In electrostaticographic reproducing apparatuses, including digital, image on image, and contact electrostatic printing apparatuses, a light image of an original to be copied is typically recorded in the form of an electrostatic latent image upon an imaging member and the latent image is subsequently rendered visible by the application of electroscopic thermoplastic resin particles and pigment particles, or toner. Electrophotographic imaging members may include imaging members (photoreceptors) which are commonly utilized in electrophotographic (xerographic) processes, in either a flexible belt or a rigid drum configuration. Other members may include flexible intermediate transfer belts that are seamless or seamed, and usually formed by cutting a rectangular sheet from a web, overlapping opposite ends, and welding the overlapped ends together to form a welded seam. These electrophotographic imaging members comprise a photoconductive layer comprising a single layer or composite layers.

The term "electrostaticographic" is generally used interchangeably with the term "electrophotographic." In addition, the terms "charge blocking layer" and "blocking layer" are generally used interchangeably with the phrase "undercoat layer."

One type of composite photoconductive layer used in xerography is illustrated in U.S. Pat. No. 4,265,990 which describes a imaging member having at least two electrically operative layers. One layer comprises a photoconductive layer which is capable of photogenerating holes and injecting the photogenerated holes into a contiguous charge transport layer (CTL). Generally, where the two electrically operative layers are supported on a conductive layer, the photoconductive layer is sandwiched between a contiguous CTL and the supporting conductive layer. Alternatively, the CTL may be sandwiched between the supporting electrode and a photoconductive layer. Imaging members having at least two electrically operative layers, as disclosed above, provide excellent electrostatic latent images when charged in the dark with a uniform negative electrostatic charge, exposed to a light image and thereafter developed with finely divided electroscopic marking particles. The resulting toner image is usually transferred to a suitable receiving member such as paper or to an intermediate transfer member which thereafter transfers the image to a member such as paper.

In the case where the charge-generating layer (CGL) is sandwiched between the CTL and the electrically conducting layer, the outer surface of the CTL is charged negatively and the conductive layer is charged positively. The CGL then should be capable of generating electron hole pair when

exposed image wise and inject only the holes through the CTL. In the alternate case when the CTL is sandwiched between the CGL and the conductive layer, the outer surface of CGL layer is charged positively while conductive layer is charged negatively and the holes are injected through from the CGL to the CTL. The CTL should be able to transport the holes with as little trapping of charge as possible. In flexible web like imaging member the charge conductive layer may be a thin coating of metal on a thin layer of thermoplastic resin.

As more advanced, higher speed electrophotographic copiers, duplicators and printers were developed, however, degradation of image quality was encountered during extended cycling. The complex, highly sophisticated duplicating and printing systems operating at very high speeds have placed stringent requirements including narrow operating limits on imaging members. For example, the numerous layers used in many modern photoconductive imaging members must be highly flexible, adhere well to adjacent layers, and exhibit predictable electrical characteristics within narrow operating limits to provide excellent toner images over many thousands of cycles. One type of multilayered imaging member that has been employed as a belt in electrophotographic imaging systems comprises a substrate, a conductive layer, an optional blocking layer, an optional adhesive layer, a CGL, a CTL and a conductive ground strip layer adjacent to one edge of the imaging layers, and an optional overcoat layer adjacent to another edge of the imaging layers. Such an imaging member may further comprise an anti-curl back coating layer on the side of the substrate opposite the side carrying the conductive layer, support layer, blocking layer, adhesive layer, CGL, CTL and other layers.

In a typical machine design, a flexible imaging member belt is mounted over and around a belt support module comprising numbers of belt support rollers, such that the top outermost charge transport layer is exposed to all electrophotographic imaging subsystems interactions. Under a normal machine imaging function condition, the top exposed charge transport layer surface of the flexible imaging member belt is constantly subjected to physical/mechanical/electrical/chemical species actions against the mechanical sliding actions of cleaning blade and cleaning brush, electrical charging devices, corona effluents exposure, developer components, image formation toner particles, hard carrier particles, receiving paper, and the like during dynamic belt cyclic motion. These machine subsystem interactions against the surface of the charge transport layer have been found to consequently cause surface contamination, scratching, abrasion-all of which can lead to rapid charge transport layer surface wear problems. Thus, a major factor limiting imaging member life in copiers and printers, is wear and how wear affects the multiple layers of the imaging member. For example, the durability of the charge transport, overcoat and anti-curl back coating (ACBC) layers, and the ability of these layers to resist wear, will greatly impact the imaging member life.

Binders of a weight that fall within a critical molecular weight range are used in current imaging members. These binders require a high molecular range so that the desired viscosity can be achieved. The viscosity level imparts high quality coating for the imaging member layers and is critical for long mechanical flexing life. Generally, uneven thickness in the layers of the photoreceptive material of the imaging member results in performance degradation of the belt. Accordingly, it is desired that each layer have a substantially uniform thickness across the web. Without these binders, the layers of the imaging member will have uneven thickness and substantially lower wear resistance, thus decreasing the over-

all life and operability of the imaging member. In addition, because certain layers of the imaging member, such as for example, the charge transport layer, the anti-curl back coating layer and the ground strip layer, can greatly impact the mechanical life of the imaging member, incorporation of the binder into such layers are desirable to increase quality and life.

The charge transport layer is a photoconductive layer that photogenerates holes and injects the photogenerated holes into an adjacent layer. The charge transport layer may also be known as a "small molecule transport layer." The small molecule dispersed in the charge transport layer help facilitate the charge transport through the layer which is important as this layer is used to maintain electron movement and prevent electrostatic charge buildup.

The ground strip layer is applied to one edge of the imaging member. Inclusion of this layer helps to promote electrical continuity with the other layers, such as the conductive layer through the hole-blocking layer.

In the production of multilayered imaging members, the drying/cooling process used to form the layers will often cause upward curling of the multiple layers. This upward curling is a consequence of thermal contraction mismatch between the CTL and the substrate support. Curling of a imaging member web is undesirable because it hinders fabrication of the web into cut sheets and subsequent welding into a belt. To offset the curling, an anti-curl back coating is applied to the backside of the flexible substrate support, opposite to the side having the charge transport layer, to render the imaging member web stock with desired flatness.

Thus, the above layers can greatly affect imaging member life but can also each act as a limiting factor if not made with specific materials. As such, incorporation of these binders into the above layers, are very important for the quality of current imaging members. However, the conventional binder commonly incorporated in the imaging members are no longer being manufactured and present supplies will be running out. Therefore, there is a need for an alternative and cost-effective binder for use with current imaging members to impart wear resistance and good coating qualities that may maintain mechanical life.

#### BRIEF SUMMARY

Embodiments include an imaging member comprising a substrate, a charge generating layer disposed on the substrate, a charge transport layer disposed on the charge generating layer, an anti-curl back coating layer disposed on the substrate opposite to the charge transport layer, and a ground strip layer disposed on one edge of the imaging member, wherein at least one of the charge transport layer, anti-curl back coating layer, and ground strip layer comprises a binder comprising bisphenol-A-polycarbonate having a high molecular weight of from about 100,000 to about 200,000 measured as polystyrene equivalents.

Another embodiment provides an imaging member, comprising a substrate, a charge generating layer disposed on the substrate, a charge transport layer disposed on the charge generating layer, an anti-curl back coating layer disposed on the substrate opposite to the charge transport layer, and a ground strip layer disposed on one edge of the imaging member, wherein at least one of the charge transport layer, anti-curl back coating layer, and ground strip layer comprises a binder comprising bisphenol-A-polycarbonate having a high molecular weight of from about 100,000 to about 200,000 and is present in at least one of the charge transport layer,

anti-curl back coating layer, and the ground strip layer from about 50 percent to about 100 percent weight of the total weight of the respective layer.

Yet another embodiment provides an image forming apparatus for forming images on a recording medium comprising an imaging member having a charge retentive surface for receiving an electrostatic latent image thereon, wherein the imaging member comprises a substrate, a charge generating layer disposed on the substrate, a charge transport layer disposed on the charge generating layer, an anti-curl back coating layer disposed on the substrate opposite to the charge transport layer, and a ground strip layer disposed on one edge of the imaging member, wherein at least one of the charge transport layer, anti-curl back coating layer, and ground strip layer comprises a binder comprising bisphenol-A-polycarbonate having a high molecular weight of from about 100,000 to about 200,000, a development component adjacent to the charge-retentive surface for applying a developer material to the charge-retentive surface, a transfer component adjacent to the charge-retentive surface for transferring the developed image from the charge-retentive surface to a copy substrate, and a fusing component adjacent to the copy substrate for fusing the developed image to the copy substrate.

#### BRIEF DESCRIPTION OF THE DRAWINGS

The above embodiments will become apparent as the following description proceeds upon reference to the following drawing:

FIG. 1 is a cross-section view of a multilayered electro-photographic imaging member of flexible belt configuration according to an embodiment.

FIG. 2 is a graphical evaluation of the electrical and cycling performance of the inventive binders compared with the conventional binder as shown through a Photo Induced Discharge Curve.

#### DETAILED DESCRIPTION

In the following description, reference is made to the accompanying drawings which form a part hereof and which illustrate several embodiments. It is understood that other embodiments may be utilized and structural and operational changes may be made without departing from the scope of the present embodiments.

The present embodiments relate to the use of a newly developed polycarbonate resin that has a molecular weight which falls within the critical molecular weight range needed to impart desirable qualities to an imaging member. The polycarbonate material also has methylene chloride solubility which makes it compatible with the \$80M worth of coating equipment Xerox now owns. The polycarbonate provides uniform coating to the layer or layers that it is incorporated into and improves mechanical robustness. The polycarbonate material has also been scaled appropriately to allow production of the desired binders in large quantities, thus effectively reducing manufacturing costs.

In accordance with embodiments, the newly developed polycarbonate binder (available from Mitsubishi Gas Chemical America, Inc.) is polymerized from bisphenol-A, which makes it less costly than most commonly available polycarbonates manufactured from bisphenol-Z. The resulting binder is comprised of poly(4,4'-isopropylidene-diphenylene)carbonate (also referred to as bisphenol-A-polycarbonate or PCA). The bisphenol-A-polycarbonate has a high molecular weight range of from about 100,000 to about 200,

000. In embodiments, the molecular weight range may be from about 170,000 to about 190,000.

The high molecular weight of the polycarbonate imparts a desired level of viscosity that provides high quality coating in the imaging members and their layers. This desired level of viscosity also is a strong contributing factor to long mechanical flexing life. In embodiments, the viscosity layer coatings comprising the polycarbonate is from about 500 cP to about 1000 cP. In other embodiments, the viscosity is from about 540 cP to about 620 cP.

The glass transition temperature (Tg) of the polycarbonate is 156.3° C., and thus very similar to that of the conventional binder. This similarity ensures that an imaging member incorporating the new polycarbonate binder will perform substantially the same as the conventional binder in the heat stress relief step. The glass transition of the layer comprising the binder is from about 150° C. to about 160° C. The polycarbonate binder is suitable for incorporation into one or more of three imaging member layers, including the charge transport layer or small molecule transport layer, the anti-curl back coating layer, and the ground strip layer. The binder may also be present in each of the three imaging member layers. For example, the binder may be present in the charge transport layer in an amount of 50 to 70 percent by weight of the total weight of the charge transport layer or present in the anticurl back coating layer in an amount of 90 to 100 percent by weight of the total weight of the anticurl back coating layer or present in the ground strip layer in an amount of 60 to 80 percent by weight of the total weight of the ground strip layer.

The embodiments of the present imaging member are utilized in an electrophotographic image forming member for use in an electrophotographic imaging process. As explained above, such image formation involves first uniformly electrostatically charging the imaging member, then exposing the charged imaging member to a pattern of activating electromagnetic radiation such as light, which selectively dissipates the charge in the illuminated areas of the imaging member while leaving behind an electrostatic latent image in the non-illuminated areas. This electrostatic latent image may then be developed at one or more developing stations to form a visible image by depositing finely divided electroscopic toner particles, for example, from a developer composition, on the surface of the imaging member. The resulting visible toner image can be transferred to a suitable receiving member, such as paper. The imaging member is then typically cleaned at a cleaning station prior to being recharged for formation of subsequent images.

Alternatively, the developed image can be transferred to another intermediate transfer device, such as a belt or a drum, via the transfer member. The image can then be transferred to the paper by another transfer member. The toner particles may be transfixed or fused by heat and/or pressure to the paper. The final receiving medium is not limited to paper. It can be various substrates such as cloth, conducting or non-conducting sheets of polymer or metals. It can be in various forms, sheets or curved surfaces. After the toner has been transferred to the imaging member, it can then be transfixed by high pressure rollers or fusing component under heat and/or pressure.

An exemplary embodiment of a multilayered electrophotographic imaging member of flexible belt configuration is illustrated in FIG. 1. The exemplary imaging member includes a support substrate 10 having an optional conductive surface layer or layers 12 (which may be referred to herein as a ground plane layer), optional if the substrate itself is conductive, a hole-blocking layer 14, an optional adhesive interface layer 16, a charge generating layer 18 and a charge

transport layer 20, and optionally one or more overcoat and/or protective layer 26. The charge generating layer 18 and the charge transport layer 20 forms an imaging layer described here as two separate layers. It will be appreciated that the functional components of these layers may alternatively be combined into a single layer.

Other layers of the imaging member may include, for example, an optional ground strip layer applied to one edge of the imaging member to promote electrical continuity with the 10 conductive layer 12 through the hole-blocking layer 14. An anti-curl back coating layer 30 of the imaging member may be formed on the backside of the support substrate 10. The conductive ground plane 12 is typically a thin metallic layer, for example a 10 nanometer thick titanium coating, deposited 15 over the substrate 10 by vacuum deposition or sputtering process. The layers 14, 16, 18, 20 and 26 may be separately and sequentially deposited on to the surface of conductive ground plane 12 of substrate 10 as solutions comprising a solvent, with each layer being dried before deposition of the 20 next.

#### The Substrate

The imaging member support substrate 10 may be opaque or substantially transparent, and may comprise any suitable organic or inorganic material having the requisite mechanical 25 properties. The entire substrate can comprise the same material as that in the electrically conductive surface, or the electrically conductive surface can be merely a coating on the substrate. Any suitable electrically conductive material can be employed. Typical electrically conductive materials 30 include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, chromium, tungsten, molybdenum, paper rendered conductive by the 35 inclusion of a suitable material therein or through conditioning in a humid atmosphere to ensure the presence of sufficient water content to render the material conductive, indium, tin, metal oxides, including tin oxide and indium tin oxide, and the like. It could be single metallic compound or dual layers 40 of different metals and/or oxides.

The substrate 10 can also be formulated entirely of an electrically conductive material, or it can be an insulating material including inorganic or organic polymeric materials, such as MYLAR, a commercially available biaxially oriented 45 polyethylene terephthalate from DuPont, or polyethylene naphthalate available as KALEDEX 2000, with a ground plane layer 12 comprising a conductive titanium or titanium/zirconium coating, otherwise a layer of an organic or inorganic material having a semiconductive surface layer, such as 50 indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic 55 considerations.

The substrate 10 may have a number of many different configurations, such as for example, a plate, a cylinder, a drum, a scroll, an endless flexible belt, and the like. In the case of the substrate being in the form of a belt, the belt can be 60 seamed or seamless.

The thickness of the substrate 10 depends on numerous factors, including flexibility, mechanical performance, and economic considerations. The thickness of the support substrate 10 may range from about 25 micrometers to about 65 3,000 micrometers. In embodiments of flexible imaging member belt preparation, the thickness of substrate 10 is from about 50 micrometers to about 200 micrometers for optimum

flexibility and to effect minimum induced imaging member surface bending stress when a imaging member belt is cycled around small diameter rollers in a machine belt support module, for example, 19 millimeter diameter rollers.

An exemplary substrate support **10** is not soluble in any of the solvents used in each coating layer solution, is optically transparent or semi-transparent, and is thermally stable up to a high temperature of about 150 oC. A typical substrate support **10** used for imaging member fabrication has a thermal contraction coefficient ranging from about 1×10-5 per oC to about 3×10-5 per oC and a Young's Modulus of between about 5×10-5 psi (3.5×10-4 Kg/cm2) and about 7×10-5 psi (4.9×10-4 Kg/cm2).

#### The Conductive Layer

The conductive ground plane layer **12** may vary in thickness depending on the optical transparency and flexibility desired for the electrophotographic imaging member. When a imaging member flexible belt is desired, the thickness of the conductive layer **12** on the support substrate **10**, for example, a titanium and/or zirconium conductive layer produced by a sputtered deposition process, typically ranges from about 2 nanometers to about 75 nanometers to allow adequate light transmission for proper back erase, and in embodiments from about 10 nanometers to about 20 nanometers for an optimum combination of electrical conductivity, flexibility, and light transmission. Generally, for rear erase exposure, a conductive layer light transparency of at least about 15 percent is desirable. The conductive layer need not be limited to metals. The conductive layer **12** may be an electrically conductive metal layer which may be formed, for example, on the substrate by any suitable coating technique, such as a vacuum depositing or sputtering technique. Typical metals suitable for use as conductive layer **12** include aluminum, zirconium, niobium, tantalum, vanadium, hafnium, titanium, nickel, stainless steel, chromium, tungsten, molybdenum, combinations thereof, and the like. Where the entire substrate is an electrically conductive metal, the outer surface can perform the function of an electrically conductive layer and a separate electrical conductive layer may be omitted. Other examples of conductive layers may be combinations of materials such as conductive indium tin oxide as a transparent layer for light having a wavelength between about 4000 Angstroms and about 9000 Angstroms or a conductive carbon black dispersed in a plastic binder as an opaque conductive layer.

The illustrated embodiment will be described in terms of a substrate layer **10** comprising an insulating material including inorganic or organic polymeric materials, such as, MYLAR with a ground plane layer **12** comprising an electrically conductive material, such as titanium or titanium/zirconium, coating over the substrate layer **10**.

#### The Hole-blocking Layer

An optional hole-blocking layer **14** may then be applied to the substrate **10** or to the layer **12**, where present. Any suitable positive charge (hole) blocking layer capable of forming an effective barrier to the injection of holes from the adjacent conductive layer **12** into the photoconductive or charge generating layer may be utilized. The charge (hole) blocking layer may include polymers, such as, polyvinylbutyral, epoxy resins, polyesters, polysiloxanes, polyamides, polyurethanes, HEMA, hydroxylpropyl cellulose, polyphosphazine, and the like, or may comprise nitrogen containing siloxanes or silanes, or nitrogen containing titanium or zirconium compounds, such as, titanate and zirconate. The hole-blocking layer should be continuous and may have a thickness in a wide range of from about 0.2 microns to about 10 micrometers depending on the type of material chosen for use in a imaging member design. Typical hole-blocking layer materials

include, for example, trimethoxysilyl propylene diamine, hydrolyzed trimethoxysilyl propyl ethylene diamine, N-beta-(aminoethyl)gamma-aminopropyl trimethoxy silane, isopropyl 4-aminobenzene sulfonyl di(dodecylbenzene sulfonyl) titanate, isopropyl di(4-aminobenzoyl)isostearoyl titanate, isopropyl tri(N-ethylaminoethylamino)titanate, isopropyl tri-anthranil titanate, isopropyl tri(N,N-dimethylaminoethylamino)titanate, titanium 4-amino benzene sulfonate oxyacetate, titanium 4-aminobenzoate isostearate oxyacetate, (gamma-aminobutyl) methyl diethoxysilane which has the formula [H2N(CH2)4]CH3Si(OCH3)2, and (gamma-aminopropyl) methyl diethoxysilane, which has the formula [H2N(CH2)3]CH3Si(OCH3)2, and combinations thereof, as disclosed, for example, in U.S. Pat. Nos. 4,338,387; 4,286,033; and 4,291,110, incorporated herein by reference in their entireties. An embodiment of a hole-blocking layer comprises a reaction product between a hydrolyzed silane or mixture of hydrolyzed silanes and the oxidized surface of a metal ground plane layer. The oxidized surface inherently forms on the outer surface of most metal ground plane layers when exposed to air after deposition. This combination enhances electrical stability at low RH. Other suitable charge blocking layer polymer compositions are also described in U.S. Pat. No. 5,244,762 which is incorporated herein by reference in its entirety. These include vinyl hydroxyl ester and vinyl hydroxy amide polymers wherein the hydroxyl groups have been partially modified to benzoate and acetate esters which are then blended with other unmodified vinyl hydroxyl ester and amide unmodified polymers. An example of such a blend is a 30 mole percent benzoate ester of poly(2-hydroxyethyl methacrylate) blended with the parent polymer poly (2-hydroxyethyl methacrylate). Still other suitable charge blocking layer polymer compositions are described in U.S. Pat. No. 4,988,597, which is incorporated herein by reference in its entirety. These include polymers containing an alkyl acrylamidoglycolate alkyl ether repeat unit. An example of such an alkyl acrylamidoglycolate alkyl ether containing polymer is the copolymer poly(methyl acrylamidoglycolate methyl ether-co-2-hydroxyethyl methacrylate).

The blocking layer **14** can be continuous or substantially continuous and may have a thickness of less than about 10 micrometers because greater thicknesses may lead to undesirably high residual voltage. In aspects of the exemplary embodiment, a blocking layer of from about 0.005 micrometers to about 2 micrometers gives optimum electrical performance. The blocking layer may be applied by any suitable conventional technique, such as, spraying, dip coating, draw bar coating, gravure coating, silk screening, air knife coating, reverse roll coating, vacuum deposition, chemical treatment, and the like. For convenience in obtaining thin layers, the blocking layer may be applied in the form of a dilute solution, with the solvent being removed after deposition of the coating by conventional techniques, such as, by vacuum, heating, and the like. Generally, a weight ratio of blocking layer material and solvent of between about 0.05:100 to about 5:100 is satisfactory for spray coating.

#### The Adhesive Interface Layer

An optional separate adhesive interface layer **16** may be provided. In the embodiment illustrated in FIG. 1, an interface layer **16** is situated intermediate the blocking layer **14** and the charge generator layer **18**. The interface layer may include a co-polyester resin. Exemplary polyester resins which may be utilized for the interface layer include polyarylatepolyvinylbutyral, such as ARDEL POLYARYLATE (U-100) commercially available from Toyota Hsutsu Inc., VITEL PE-100, VITEL PE-200, VITEL PE-200D, and VITEL PE-222, all from Bostik, 49,000 polyester from Rohm

Hass, polyvinyl butyral, and the like. The adhesive interface layer **16** may be applied directly to the hole-blocking layer **14**. Thus, the adhesive interface layer **16** in embodiments is in direct contiguous contact with both the underlying hole-blocking layer **14** and the overlying charge generator layer **18** to enhance adhesion bonding to provide linkage. In yet other embodiments, the adhesive interface layer **16** is entirely omitted.

Any suitable solvent or solvent mixtures may be employed to form a coating solution of the polyester for the adhesive interface layer **16**. Typical solvents include tetrahydrofuran, toluene, monochlorobenzene, methylene chloride, cyclohexanone, and the like, and mixtures thereof. Any other suitable and conventional technique may be used to mix and thereafter apply the adhesive layer coating mixture to the hole-blocking layer. Typical application techniques include spraying, dip coating, roll coating, wire wound rod coating, and the like. Drying of the deposited wet coating may be effected by any suitable conventional process, such as oven drying, infra red radiation drying, air drying, and the like.

The adhesive interface layer **16** may have a thickness of from about 0.01 micrometers to about 900 micrometers after drying. In embodiments, the dried thickness is from about 0.03 micrometers to about 1 micrometer.

#### The Charge Generating Layer

The charge generating layer **18** may thereafter be applied to the adhesive layer **16**. Any suitable charge generating binder including a charge generating/photoconductive material, which may be in the form of particles and dispersed in a film forming binder, such as an inactive resin, may be utilized. Examples of charge generating materials include, for example, inorganic photoconductive materials such as amorphous selenium, trigonal selenium, and selenium alloys selected from the group consisting of selenium-tellurium, selenium-tellurium-arsenic, selenium arsenide and mixtures thereof, and organic photoconductive materials including various phthalocyanine pigments such as the X-form of metal free phthalocyanine, metal phthalocyanines such as vanadyl phthalocyanine and copper phthalocyanine, hydroxy gallium phthalocyanines, chlorogallium phthalocyanines, titanyl phthalocyanines, quinacridones, dibromo anthanthrone pigments, benzimidazole perylene, substituted 2,4-diamino-triazines, polynuclear aromatic quinones, and the like dispersed in a film forming polymeric binder. Selenium, selenium alloy, benzimidazole perylene, and the like and mixtures thereof may be formed as a continuous, homogeneous charge generating layer. Benzimidazole perylene compositions are well known and described, for example, in U.S. Pat. No. 4,587,189, the entire disclosure thereof being incorporated herein by reference. Multi-charge generating layer compositions may be utilized where a photoconductive layer enhances or reduces the properties of the charge generating layer. Other suitable charge generating materials known in the art may also be utilized, if desired. The charge generating materials selected should be sensitive to activating radiation having a wavelength between about 400 and about 900 nm during the imagewise radiation exposure step in an electrophotographic imaging process to form an electrostatic latent image. For example, hydroxygallium phthalocyanine absorbs light of a wavelength of from about 370 to about 950 nanometers, as disclosed, for example, in U.S. Pat. No. 5,756,245.

Any suitable inactive resin materials may be employed as a binder in the charge generating layer **18**, including those described, for example, in U.S. Pat. No. 3,121,006, the entire disclosure thereof being incorporated herein by reference. Typical organic resinous binders include thermoplastic and thermosetting resins such as one or more of polycarbonates,

polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like. Another film-forming polymer binder is PCZ-400 (poly (4,4'-dihydroxy-diphenyl-1-1-cyclohexane) which has a viscosity-molecular weight of 40,000 and is available from Mitsubishi Gas Chemical Corporation.

The charge generating material can be present in the resinous binder composition in various amounts. Generally, from about 5 percent by volume to about 90 percent by volume of the charge generating material is dispersed in about 10 percent by volume to about 95 percent by volume of the resinous binder, and more specifically from about 20 percent by volume to about 60 percent by volume of the charge generating material is dispersed in about 40 percent by volume to about 80 percent by volume of the resinous binder composition.

The charge generating layer **18** containing the charge generating material and the resinous binder material generally ranges in thickness of from about 0.1 micrometer to about 5 micrometers, for example, from about 0.3 micrometers to about 3 micrometers when dry. The charge generating layer thickness is generally related to binder content. Higher binder content compositions generally employ thicker layers for charge generation.

#### The Charge Transport Layer

The charge transport layer **20** is thereafter applied over the charge generating layer **18** and may include any suitable transparent organic polymer or non-polymeric material capable of supporting the injection of photogenerated holes or electrons from the charge generating layer **18** and capable of allowing the transport of these holes/electrons through the charge transport layer to selectively discharge the surface charge on the imaging member surface. In one embodiment, the charge transport layer **20** not only serves to transport holes, but also protects the charge generating layer **18** from abrasion or chemical attack and may therefore extend the service life of the imaging member. The charge transport layer **20** can be a substantially non-photoconductive material, but one which supports the injection of photogenerated holes from the charge generation layer **18**. The layer **20** is normally transparent in a wavelength region in which the electrophotographic imaging member is to be used when exposure is effected therethrough to ensure that most of the incident radiation is utilized by the underlying charge generating layer **18**. The charge transport layer should exhibit excellent optical transparency with negligible light absorption and negligible charge generation when exposed to a wavelength of light useful in xerography, e.g., 400 to 900 nanometers. In the case when the imaging member is prepared with the use of a transparent substrate **10** and also a transparent or partially transparent conductive layer **12**, image wise exposure or erase may be accomplished through the substrate **10** with all light passing through the back side of the substrate. In this case, the materials of the layer **20** need not transmit light in the wavelength region of use if the charge generating layer **18** is sandwiched between the substrate and the charge transport

## 11

layer **20**. The charge transport layer **20** in conjunction with the charge generating layer **18** is an insulator to the extent that an electrostatic charge placed on the charge transport layer is not conducted in the absence of illumination. The charge transport layer **20** should trap minimal charges as the charge passes through it during the discharging process.

The high molecular weight bisphenol-A-polycarbonate may be present in the charge transport layer as a binder. The bisphenol-A-polycarbonate binder may be present in an amount of from about 40 to about 80 percent by weight of the total weight of the charge transport layer. In embodiments, the bisphenol-A-polycarbonate binder may also be present in an amount of from about 50 to about 70 percent by weight of the total weight of the charge transport layer.

The charge transport layer **20** may include any suitable charge transport molecule or activating compound useful as an additive molecularly dispersed in an electrically inactive polymeric material to form a solid solution and thereby making this material electrically active. The charge transport molecule may be added to a film forming polymeric material which is otherwise incapable of supporting the injection of photogenerated holes from the charge generation material and incapable of allowing the transport of these holes through. This addition converts the electrically inactive polymeric material to a material capable of supporting the injection of photogenerated holes from the charge generation layer **18** and capable of allowing the transport of these holes through the charge transport layer **20** in order to discharge the surface charge on the charge transport layer. The charge transport molecule typically comprises small molecules of an organic compound which cooperate to transport charge between molecules and ultimately to the surface of the charge transport layer, for example, (N,N'-diphenyl-N,N'-bis(3-methylphenyl)-1,1'-biphenyl)-4,4'-diamine. The charge transport molecule or components may be, for example, represented by the following structure:



wherein X is selected from the group consisting of alkyl, alkoxy, and halogen. In embodiments the alkyl and alkoxy contain from about 1 to about 12 carbon atoms. In other embodiments, the alkyl contains from about 1 to about 5 carbon atoms. In yet another embodiment, the alkyl is methyl.

In the embodiments, any suitable charge transporting polymer may also be used in the charge transporting layer. The charge transporting polymer should be insoluble in the alcohol solvent employed to apply the charge transport layer.

Any suitable electrically inactive resin binder insoluble in the alcohol solvent may be used to apply the charge transport layer. Typical inactive resin binders include polycarbonate resin, polystyrene, polyester, polyarylate, polyacrylate, polyether, polysulfone, and the like. Molecular weights can vary, for example, from about 20,000 to about 150,000. Examples of binders include polycarbonates such as poly(4,4'-isopropylidene-diphenylene)carbonate (also referred to as bisphenol-A-polycarbonate), poly(4,4'-cyclohexylidene-diphenylene)carbonate (referred to as bisphenol-Z polycarbonate),

## 12

poly(4,4'-isopropylidene-3,3'-dimethyl-diphenyl)carbonate (also referred to as bisphenol-C-polycarbonate) and the like.

Any suitable and conventional technique may be used to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like.

Other exemplary charge transport molecules include aromatic polyamines, such as aryl diamines and aryl triamines. Exemplary aromatic diamines include N,N'-diphenyl-N,N'-bis(alkylphenyl)-1,1'-biphenyl-4,4'-diamines; (N,N'-diphenyl-N,N'-bis[3-methylphenyl]-1,1'-biphenyl)-4,4'-diamine; N,N'-diphenyl-N,N'-bis(chlorophenyl)-1,1'-biphenyl-4,4'-diamine; and N,N'-bis-(4-methylphenyl)-N,N'-bis(4-ethylphenyl)-1,1'-3,3'-dimethylbiphenyl)-4,4'-diamine, N,N'-bis-(3,4-dimethylphenyl)-4,4'-biphenyl amine, and combinations thereof.

Further suitable charge transport molecules include pyrazolines, such as 1-[lepidyl-(2)]-3-(p-diethylaminophenyl)-5-(p-diethylaminophenyl)pyrazoline, as described, for example, in U.S. Pat. Nos. 4,315,982, 4,278,746, 3,837,851, and 6,214,514, substituted fluorene charge transport molecules, such as 9-(4'-dimethylaminobenzylidene)fluorene, as described in U.S. Pat. Nos. 4,245,021 and 6,214,514, oxadiazole transport molecules, such as 2,5-bis(4-diethylaminophenyl)-1,3,4-oxadiazole, pyrazoline, imidazole, triazole, as described, for example in U.S. Pat. No. 3,895,944, hydrazones, such as p-diethylaminobenzaldehyde (diphenylhydrazone), as described, for example in U.S. Pat. Nos. 4,150,987 4,256,821, 4,297,426, 4,338,388, 4,385,106, 4,387,147, 4,399,207, 4,399,208, 6,124,514, and tri-substituted methanes, such as alkyl-bis(N,N-dialkylaminoaryl)methanes, as described, for example, in U.S. Pat. No. 3,820,989. The disclosures of all of these patents are incorporated herein by reference in their entireties.

The concentration of the charge transport molecule in layer **20** may be, for example, at least about 5 weight percent and may comprise up to about 60 weight percent. The concentration or composition of the charge transport molecule may vary through layer **20**, as described, for example, in U.S. application Ser. No. 10/736,864, filed Dec. 16, 2003, entitled "Imaging Members," by Anthony M. Horgan, et al., which was published on Jul. 1, 2004, as Application Serial No. 2004/0126684; U.S. application Ser. No. 10/320,808, filed Dec. 16, 2002, entitled "Imaging Members," by Anthony M. Horgan, et al., which was published on Jun. 17, 2004, as Application Serial No. 2004/0115545, and U.S. application Ser. No. 10/655,882, filed Sep. 5, 2003, entitled "Dual charge transport layer and photoconductive imaging member including the same," by Damodar M. Pai, et al., which was published on Mar. 10, 2005 as Application Serial No. 2005/0053854, the disclosures of which are incorporated herein by reference in their entireties.

In one exemplary embodiment, the charge transport layer **20** comprises an average of about 10-60 weight percent N,N'-diphenyl-N,N'-bis(3-methylphenyl)-1,1'-biphenyl-4,4'-diamine, such as from about 30-50 weight percent N,N'-diphenyl-N,N'-bis(3-methylphenyl)-1,1'-biphenyl-4,4'-diamine.

The charge transport layer **20** is an insulator to the extent that the electrostatic charge placed on the charge transport layer is not conducted in the absence of illumination at a rate sufficient to prevent formation and retention of an electrostatic latent image thereon. In general, the ratio of the thickness of the charge transport layer **20** to the charge generator

## 13

layer 18 is maintained from about 2:1 to about 200:1 and in some instances as great as about 400:1.

Additional aspects relate to the inclusion in the charge transport layer 20 of variable amounts of an antioxidant, such as a hindered phenol. Exemplary hindered phenols include octadecyl-3,5-di-tert-butyl-4-hydroxyhydrocinnamate, available as IRGANOX 1-1010 from Ciba Specialty Chemicals. The hindered phenol may be present as up to about 10 weight percent based on the concentration of the charge transport molecule. Other suitable antioxidants are described, for example, in above-mentioned U.S. application Ser. No. 10/655,882 incorporated by reference.

In one specific embodiment, the charge transport layer 20 is a solid solution including a charge transport molecule, such as N,N'-diphenyl-N,N'-bis(3-methylphenyl)-1,1'-biphenyl-4,4'-diamine, molecularly dissolved in a polycarbonate binder, the binder being either a poly(4,4'-isopropylidene diphenyl carbonate) or a poly(4,4'-diphenyl-1,1'-cyclohexane carbonate).

The thickness of the charge transport layer 20 can be from about 5 micrometers to about 200 micrometers, e.g., from between about 15 micrometers and about 40 micrometers. The charge transport layer may comprise dual layers or multiple layers with different concentration of charge transporting components.

Other layers such as conventional ground strip layer 38 including, for example, conductive particles dispersed in a film forming binder may be applied to one edge of the imaging member to promote electrical continuity to the conductive layer 12. The ground strip layer 38 may include any suitable film forming polymer binder and electrically conductive particles. Typical ground strip materials include those enumerated in U.S. Pat. No. 4,664,995, the entire disclosure of which is incorporated by reference herein.

An overcoat layer 26 may also be utilized to provide imaging member surface protection, improved cleanability, reduced friction, as well as improve resistance to abrasion.

#### The Overcoat Layer

Additional aspects relate to overcoat layers that may comprise a dispersion of nanoparticles, such as silica, metal oxides, ACUMIST (waxy polyethylene particles), polytetrafluoroethylene (PTFE), and the like. The nanoparticles may be used to enhance the lubricity, scratch resistance, and wear resistance of the overcoat layer 26. In embodiments, the nanoparticles are comprised of nano polymeric gel particles of crosslinked polystyrene-n-butyl acrylate which is dispersed or doped into a binder polymer matrix.

In the larger printing apparatuses, adequate reduction of friction largely removes the need for additional members or components, subsequently reducing the cost of the imaging member. The overcoat layer 26 provides an outer level of protection on the imaging member and may help bolster wear resistance and scratch resistance of the charge transport layer in the print engine.

The high molecular weight bisphenol-A-polycarbonate may be present in the overcoat layer as a binder. The bisphenol-A-polycarbonate binder may be present in an amount of from about 50 to about 98 percent by weight of the total weight of the overcoat layer. In embodiments, the bisphenol-A-polycarbonate binder may also be present in an amount of from about 80 to about 90 percent by weight of the total weight of the overcoat layer.

Any suitable and conventional technique may be utilized to form and thereafter apply the overcoat layer mixture to the imaging layer. Typical application techniques include, for example extrusion coating, draw bar coating, roll coating, wire wound rod coating, and the like. The overcoat layer 26

## 14

may be formed in a single coating step or in multiple coating steps. Drying of the deposited coating may be effected by any suitable conventional technique such as oven drying, infra red radiation drying, air drying and the like. The thickness of the dried overcoat layer may depend upon the abrasiveness of the charging, cleaning, development, transfer, etc. system employed and can range up to about 10 microns. In these embodiments, the thickness can be between about 0.5 microns and about 10 microns in thickness, or be between about 1 micron and about 5 microns. An overcoat can have a thickness of at most 3 microns for insulating matrices and at most 6 microns for semi-conductive matrices. However, the thickness of overcoat layers may be outside this range.

#### The Ground Strip

The ground strip 38 may comprise a film forming polymer binder and electrically conductive particles. Any suitable electrically conductive particles may be used in the electrically conductive ground strip layer. Typical electrically conductive particles include carbon black, graphite, copper, silver, gold, nickel, tantalum, chromium, zirconium, vanadium, niobium, indium tin oxide and the like. The electrically conductive particles may have any suitable shape. Typical shapes include irregular, granular, spherical, elliptical, cubic, flake, filament, and the like. In embodiments, the electrically conductive particles have a particle size less than the thickness of the electrically conductive ground strip layer 38 to avoid an electrically conductive ground strip layer 38 having an excessively irregular outer surface.

The high molecular weight bisphenol-A-polycarbonate may be present in the ground strip layer as a binder. The bisphenol-A-polycarbonate binder may be present in an amount of from about 50 to about 85 percent by weight of the total weight of the ground strip layer. In embodiments, the bisphenol-A-polycarbonate binder may also be present in an amount of from about 65 to about 70 percent by weight of the total weight of the ground strip layer.

An average particle size of less than about 10 micrometers generally avoids excessive protrusion of the electrically conductive particles at the outer surface of the dried ground strip layer and ensures relatively uniform dispersion of the particles throughout the matrix of the dried ground strip layer. The concentration of the conductive particles to be used in the ground strip depends on factors such as the conductivity of the specific conductive particles utilized. In addition, silica particles are typically included in the ground strip layer 38 to improve wear. The ground strip layer 38 may have a thickness from about 7 micrometers to about 42 micrometers, or from about 14 micrometers to about 27 micrometers.

#### The Anti-curl Back Coating Layer

In some cases, an anti-curl back coating may be applied to the surface of the substrate opposite to that bearing the photoconductive layer to provide flatness and/or abrasion resistance where a web configuration imaging member is fabricated. These overcoatings and anti-curl back coating layers are well known in the art, and can comprise thermoplastic organic polymers or inorganic polymers that are electrically insulating or slightly semiconductive. The thickness of anti-curl back coating layers is generally sufficient to balance substantially the total forces of the layer or layers on the opposite side of the substrate layer. An example of an anti-curl back coating layer is described in U.S. Pat. No. 4,654,284, the disclosure of which is totally incorporated herein by reference. A thickness of from about 70 to about 160 micrometers is a typical range for flexible imaging members, although the thickness can be outside this range.

Because conventional anti-curl back coating formulations often suffer from electrostatic charge build up due to contact

## 15

friction between the anti-curl layer and the backer bars, which increases the friction and wear, incorporation of nano polymeric gel particles into the anti-curl back coating layer substantially eliminates this occurrence. In addition to reducing the electrostatic charge build up and reducing wear in the layer, the nano polymeric gel particles may be used to enhance the lubricity, scratch resistance, and wear resistance of the anti-curl back coating layer 30. In embodiments, the nano polymeric gel particles are comprised of crosslinked polystyrene-n-butyl acrylate, which is dispersed or doped into a binder polymer matrix.

All the patents and applications referred to herein are hereby specifically, and totally incorporated herein by reference in their entirety in the instant specification.

## EXAMPLES

The examples set forth hereinbelow are being submitted to illustrate embodiments of the present disclosure. These examples are intended to be illustrative only and are not intended to limit the scope of the present disclosure. Also, parts and percentages are by weight unless otherwise indicated. Comparative examples and data are also provided.

## Example 1

The polycarbonate binder has was coated on trigonal selenium generator layers, hydroxygallium generator layers, and bisphenol-Z-polycarbonate generator layers. The inventive layers were compared with a control layer with the conventional binder. The comparison is shown in Table 1.

TABLE 1

| Molecular weight and viscosity - 3 lots compared to Control |           |       |       |       |     |           |
|-------------------------------------------------------------|-----------|-------|-------|-------|-----|-----------|
| Sample Name                                                 | Mw (kpse) | Mn    | Mz    | Mp    | PD  | Viscosity |
| PCA lot 4HF1212                                             | 180.4     | 109.5 | 271.2 | 165.4 | 1.6 | 910       |
| PCA lot 5BF2262                                             | 171.3     | 102.9 | 254.5 | 159.5 | 1.7 | 780       |
| PCA lot 5CF0162                                             | 185.2     | 117.5 | 272.9 | 164.2 | 1.6 | 950       |
| Makrolon 5705 Control                                       | 145.0     | 74.8  | 243.0 | 128.2 | 1.9 | 650-950   |

The electrical and cycling performance of the above were compared to the conventional binder and shown to be equivalent to that of the conventional binder, as shown in FIG. 2. At full-scale production roll coating, the high molecular weight bisphenol-A-polycarbonate binder was coated on both the STML and the ACBC layers of test imaging members and all quality control standards of the conventional binder were met.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. An imaging member, comprising:  
a substrate;  
a charge generating layer disposed on the substrate;  
a charge transport layer disposed on the charge generating layer;

## 16

an anti-curl back coating layer disposed on the substrate opposite to the charge transport layer; and  
a ground strip layer disposed on an edge of the imaging member;

5 wherein at least one of the charge transport layer, anti-curl back coating layer, and ground strip layer comprises a binder comprising bisphenol-A-polycarbonate having a high molecular weight of from about 170,000 to about 190,000; and  
10 wherein the viscosity of the layer coating comprising bisphenol-A-polycarbonate is from about 500 cP to about 1000 cP.

2. The imaging member of claim 1, wherein the bisphenol-A-polycarbonate is present in the binder in an amount of from 15 about 50 percent to about 100 percent weight of the total weight of the binder.

20 3. The imaging member of claim 1, wherein the binder is present in at least one of the charge transport layer, anti-curl back coating layer, and the ground strip layer from about 50 percent to about 100 percent weight of the total weight of the respective layer.

25 4. The imaging member of claim 3, wherein the binder is present in the charge transport layer in an amount of 50 to 70 percent by weight of the total weight of the charge transport layer.

5. The imaging member of claim 3, wherein the binder is present in the anti-curl back coating layer in an amount of 90 to 100 percent by weight of the total weight of the anti-curl back coating layer.

30 6. The imaging member of claim 3, wherein the binder is present in the ground strip layer in an amount of 60 to 80 percent by weight of the total weight of the ground strip layer.

7. The imaging member of claim 1, wherein the viscosity of the layer coating comprising bisphenol-A-polycarbonate is from about 540 cP to about 620 cP.

35 8. The imaging member of claim 1, wherein the glass transition of the layer comprising the binder is from about 150° C. to about 160° C.

40 9. The imaging member of claim 1, wherein the binder is present in each of the first charge transport layer, anti-curl back coating layer and ground strip layer.

10. The imaging member of claim 1, wherein the binder is polymerized from bisphenol A.

45 11. An imaging member, comprising:  
a substrate;  
a charge generating layer disposed on the substrate;  
a charge transport layer disposed on the charge generating layer;  
an anti-curl back coating layer disposed on the substrate opposite to the charge transport layer; and  
a ground strip layer disposed on one edge of the imaging member,

50 wherein at least one of the charge transport layer, anti-curl back coating layer, and ground strip layer comprises a binder comprising bisphenol-A-polycarbonate having a high molecular weight of from about 170,000 to about 190,000, and is present in at least one of the charge transport layer, anti-curl back coating layer, and the ground strip layer from about 50 percent to about 100 percent weight of the total weight of the respective layer; and

55 60 wherein the viscosity of the layer coating comprising bisphenol-A-polycarbonate is from about 500 cP to about 1000 cP.

65 12. An image forming apparatus for forming images on a recording medium comprising:

**17**

an imaging member having a charge retentive surface for receiving an electrostatic latent image thereon, wherein the imaging member comprises  
 a substrate;  
 a charge generating layer disposed on the substrate;  
 a charge transport layer disposed on the charge generating layer;  
 an anti-curl back coating layer disposed on the substrate opposite to the charge transport layer; and  
 a ground strip layer disposed on one edge of the imaging member,  
 wherein at least one of the charge transport layer, anti-curl back coating layer, and ground strip layer comprises a binder comprising bisphenol-A-polycarbonate having a high molecular weight of from about 170,000 to about 190,000;  
 a development component adjacent to the charge-retentive surface for applying a developer material to the charge-retentive surface;  
 a transfer component adjacent to the charge retentive-surface for transferring the developed image from the charge-retentive surface to a copy substrate; and  
 a fusing component adjacent to the copy substrate for fusing the developed image to the copy substrate; and  
 wherein the viscosity of the layer coating comprising bisphenol-A-polycarbonate is from about 500 cP to about 1000 cP.

10

15

20

25

**18**

13. The image forming apparatus of claim 12, wherein the bisphenol-A-polycarbonate is present in the binder in an amount of from about 50 percent to about 100 percent weight of the total weight of the binder.

14. The image forming apparatus of claim 12, wherein the binder is present in at least one of the charge transport layer, anti-curl back coating layer, and the ground strip layer from about 50 percent to about 100 percent weight of the total weight of the respective layer.

15. The image forming apparatus of claim 12, wherein the viscosity of the layer coating comprising bisphenol-A-polycarbonate is from about 540 cP to about 620 cP.

16. The image forming apparatus of claim 12, wherein the glass transition of the layer comprising the binder is from about 150° C. to about 160° C.

17. The image forming apparatus of claim 12, wherein the binder is present in each of the first charge transport layer, anti-curl back coating layer and ground strip layer.

18. The image forming apparatus of claim 17, wherein the binder is present in each of the first charge transport layer, anti-curl back coating layer and ground strip layer in an amount of from about 50 percent to about 100 percent weight of the total weight of the binder.

\* \* \* \* \*